# EUROPEAN PATENT SPECIFICATION

(11) **EP 2 082 096 B1**
(45) Date of publication and mention of the grant of the patent: **20.02.2013**
(21) Application number: 07808867.1
(22) Date of filing: 06.09.2007
(51) Int. Cl.: D21C 9/14

(54) **BLEACHING OF PULP**
ZELLSTOFFBLEICHE
BLANCHIMENT DE LA PÂTE À PAPIER

(30) Priority: 11.10.2006 EP 06122119
(43) Date of publication of application: 29.07.2009
(73) Proprietor: Akzo Nobel N.V., 6800 SB Arnhem (NL); EKA Chemicals AB, 445 80 Bohus (SE)
(72) Inventor: BJÖRKLUND, Magnus, 831 75 Östersund (SE); GRESCHIK, Thomas, Christopher, 438 35 Landvetter (SE); FÄGERSTEN, Håkan, 442 60 Kode (SE)
(74) Representative: Schalkwijk, Pieter Cornelis
(86) International application number: PCT/SE2007/050630
(87) International publication number: WO 2008/044988

(56) References cited:
- EP-A1- 0 940 498
- EP-A2- 1 270 805
- US-A- 3 501 374
- US-A- 5 030 324
- US-A- 5 268 075
- US-A1- 2006 201 642
- US-B1- 6 776 876

## Description

The present invention relates to a bleaching process which decreases the brightness reversion or yellowing of an ECF bleached pulp.

### Background of the invention

In the art of bleaching, the target is to provide high and stable brightness levels. However, brightness reversion or yellowing of pulp occurs to varying extent during storage and transportation to the paper mill depending on e.g. temperature, humidity, wood species, cooking conditions and bleaching sequence. It is therefore important to perform the bleaching so that the brightness reversion becomes as low as possible. EP-A-0 940 498 discloses a bleaching process using three chlorine dioxide stages.

In the paper "How to Improve Brightness Stability of ECF bleached Softwood and Hardwood Kraft Pulp", Suess, H.U. et al, 2004, APPITA Conference, Canberra, a standard elemental chlorine free (ECF) bleaching sequence is disclosed. The bleached pulp obtained from this sequence may, however, suffer from considerable brightness reversion. Also The Ljungberg Textbook, Pulp Technology, 2004 generally discloses ECF bleaching in which brightness reversion may suffer from considerable brightness reversion. It would thus be of interest to provide a process further improving the brightness stability. The present invention intends to provide such process, particularly for decreasing the brightness reversion of pulps derived from an alkaline pulping process with a certain content of hexenuronic acid prior to the final bleaching stage.

### The invention

The present invention relates to a process of bleaching pulp derived from an alkaline pulping process having a hexenuronic acid content prior to the final bleaching stage from 1 to 80 mmol/kg dry pulp, said process comprising three chlorine dioxide stages D0, D1, and D2, wherein the chlorine dioxide charges based on the total chlorine dioxide charge in
a) D0 is from 40 to 60 %;
b) D1 is from to 55 %;
c) D2 is from 4 to 20 %, and wherein the final chlorine dioxide stage D2 is performed at a pH from 2 to 4.5.

The pulp to be bleached may be derived from lignocellulose-containing material which may comprise e.g. wood logs, finely-divided raw materials, and woody materials, such as wood particles and non-wood such as fibres of annual or perennial plants. The woody raw material can be derived from hardwood or softwood species, such as birch, beech, aspen, alder, eucalyptus, maple, acacia, mixed tropical hardwood, pine, fir, hemlock, larch, spruce, and mixtures thereof. Non-wood plant raw material can be provided from e.g. straws of grain crops, reed canary grass, reeds, flax, hemp, kenaf, jute, ramie, sisal, abaca, coir, bamboo, bagasse or combinations thereof. However, also pulp derived from recycled pulp may be used, either separately or in mixtures with virgin pulps. The pulp can be a chemical pulp, produced using an alkaline pulping process, for example sulphate, soda processes or modifications thereof with optional additives such as anthraquinone, e.g. the soda anthraquinone (AQ) pulping process. The chemical pulp obtainable from lignocellulose-containing materials may be subjected to one or more oxygen treatment stages subsequent to the pulping process. The process can be applied to chemically digested pulps having an initial kappa number, i.e. a kappa number after digestion but before oxygen delignification, in the range from 5 to 40, for example from 8 to 30, or from 8 to 25 The referred kappa number is measured according to the ISO 302 Standard Method.

According to one embodiment, the content of hexenuronic acids in the bleached pulp prior to the final bleaching stage is from 5 to 80 or from 5 to 25, or from 5 to 15 mmol/kg dry pulp.

According to one embodiment, the pH of the first chlorine dioxide bleaching stage ranges from 2 to 4, for example from 2.5 to 3.5. According to one embodiment, the pH of the second chlorine dioxide bleaching stage ranges from 2.5 to 4.5, for example from 3 to 4. According to one embodiment, the pH of the final chlorine dioxide bleaching stage ranges from 2 to 3.5, such as from 2 to 3.4 or from 2 to 3.3 or from 2.5 to 3, or any other sub-range within the range from 2.5 to 4.5.

According to one embodiment, the temperature of the first chlorine dioxide bleaching stage ranges from 40 to 90, for example from 50 to 80 or from 55 to 70°C. According to one embodiment, the temperature of the second chlorine dioxide bleaching stage ranges from 70 to 90, for example from 80 90°C. According to one embodiment, the temperature of the final chlorine dioxide bleaching stage ranges from 80 to 100, for example from 85 to 100, or from 87 to 100 °C.

According to one embodiment, the pulp consistency in the chlorine dioxide bleaching stages ranges from 1 to 40, for example from 3 to 30 or from 5 to 15 wt%.

According to one embodiment, the charge of chlorine dioxide charge based on the total chlorine dioxide charge in D0 is from 45 to 55, for example from 45 to 50, or from 45 to 48 %. According to one embodiment, the charge of chlorine dioxide charge based on the total chlorine dioxide charge in D1 is from 35 to 50, for example from 40 to 50, or from 45 to 50 %. According to one embodiment, the charge of chlorine dioxide charge based on the total chlorine dioxide charge in D2 is from 5 to 15, for example from 5 to 12, or from 5 to 10%.

According to one embodiment, the retention time of the first chlorine dioxide bleaching stage is from 20 to 60, for example from 30 to 50, or from 35 to 45 minutes. According to one embodiment, the retention time of the second chlorine dioxide bleaching stage is from 60 to 240, for example from 60 to 120, or from 60 to 90 minutes. According to one embodiment, the retention time in the final chlorine dioxide bleaching stage is from 90 to 360, for example from 110 to 240, or from 110 to 180 minutes. According to one embodiment, the bleaching process may comprise besides chlorine dioxide stages for example ozone, peracid, oxygen and/or peroxide-containing, as well as enzyme-containing bleaching stages either in addition to the sequence of three chlorine dioxide stages or substituting any of the initial chlorine dioxide stages. According to one embodiment, also washing and/or extraction stages, acidification and/or chelating agent stages may be present in the bleaching process preceeding, between and/or subsequent to any bleaching stages.

According to one embodiment, chlorine dioxide and chelating agent stages can be carried out without any make-up chemicals added, as both stages can be performed at similar pH ranges.

According to one embodiment, a chelating agent stage is carried out essentially in absence of chlorine dioxide, as essentially most of the chlorine dioxide is washed away by the washing stage.

According to one embodiment, if exceptionally an acid is added to the treatment with the chelating agent, an acid readily available in the pulp mill may be employed.

According to one embodiment, for example subsequent to treatment with a chelating agent, the pulp can be bleached with a peroxide-containing compound which can be an inorganic peroxide compound such as hydrogen peroxide or peroxomonosulphuric acid (caro's acid) or an inorganic peroxide compound like aliphatic peracids and aromatic peracids and salts thereof. Suitable organic peroxides are peracetic acid and performic acid. For example, the peroxide-containing compound is hydrogen peroxide or a mixture of hydrogen peroxide and peracetic acid commonly referred to as equilibrium peracetic acid. When hydrogen peroxide is used the pH of the pulp suspension is suitably 7, for example in the range from 7 to 13, from 8 to 12, or from 9.5 to 11.5. The temperature of the hydrogen peroxide bleaching may be from 30 to 130, for example from 50 to 100, or from 50 to 90 °C. The length of the hydrogen peroxide treatment may be from 3 to 960, for example from 10 to 360, or from 60 to 240 minutes. Usually the amount of added hydrogen peroxide is from 1 to 60, for example from 6 to 50, or from 13 to 40 kg per tonne dry pulp. Other bleaching agents may be added to the hydrogen peroxide bleaching stage such as oxygen.

According to one embodiment, the bleaching process comprises an ECF (Elemental Chlorine Free) or a substantially ECF sequence, for example according to the following sequence: D0(OP)D1nD2, where D0, D1, and D2 indicate three chlorine dioxide (D) stages, OP indicates an oxygen-containing peroxide stage, and n indicates a neutral washing stage. According to one embodiment, the bleached pulp is subsequently treated as an aqueous suspension prior to papermaking by dewatering and drying said suspension, wherein the pH of the suspension to be treated ranges from 6.5 to 12. The bleached pulp may be further treated as set out in US appl.11/847374.

According to one embodiment, the invention also relates to a bleached pulp obtainable by the process defined herein.

The invention being thus described, it will be obvious that the same may be varied in many ways. Such variations are not to be regarded as a departure from the gist and scope of the present invention, and all such modifications as would be obvious to one skilled in the art are intended to be included within the scope of the claims. The following examples will further illustrate how the described invention may be performed without limiting the scope of it.

All parts and percentages refer to part and percent by weight, if not otherwise stated.

### Examples

The experiments were carried out employing an industrial oxygen-delignified eucalyptus pulp. The characteristics of the oxygen-delignified pulp is shown in table 1. The pulp could be characterized as a low bleaching chemical demand pulp with high content of hexenuronic acid (HexA). The pulp had an unbleached kappa number of 10.7 and required 1.5 kg/t H₂O₂ and 27 kg/t ClO₂ in the sequence D0(OP)D1nD2 to reach the brightness target 90.5% ISO.

**Table 1: Oxygen delignified eucalyptus pulp**

| Kappa number | ISO Brightness (%) | Viscosity dm³/kg | Hexenuronic acid mmol/kg |
|---|---|---|---|
| 10.7 | 58.9 | 1030 | 71 |

The aim of the experiments was to improve a standard ECF sequence, D0(OP)D1nD2, in view of brightness reversion within the limitations of an existing mill. The same total dosage of chlorine dioxide was made in all experiments.
The conditions in the D1 and D2 stages and the distribution of chlorine dioxide were varied whereas the conditions in the D0 and (OP) stages were kept constant. The retention time and temperature in the D0 stage were 45 minutes and 60°C. The (OP) stage was performed at a pressure of 0.5 MPa, a retention time of 60 minutes, a temperature of 80°C and a final pH between 11.6 and 11.9. The hydrogen peroxide (H₂O₂) dosage was 1.5 kg/t on oven dry pulp in all experiments. The pulp and chemicals were mixed at 10 wt% pulp consistency and distributed uniformly in polypropylene bags, the atmosphere of which was saturated with oxygen. The plastic bags were sealed and placed in autoclaves which were pressurized with oxygen. The chlorine dioxide dosages were given as active chlorine. The consistency was 10 wt% in all bleaching stages. All non-pressurised stages were carried out in sealed plastic polyethylene bags.
After each bleaching stage, the pulp was washed with distilled water. In the neutral wash stage (n) between the D1 and D2 stages, the pH was adjusted to between 7 and 10 with NaOH. The kappa number and ISO brightness were determined according to ISO 302 and ISO 2470 respectively. The hexenuronic acid was determined by acidic hydrolysis of the pulp in a formate buffer followed by UV analysis of the 2-furoic acid formed in the hydrolysate.
The accelerated heat-induced brightness reversion was evaluated as humid brightness reversion. The "humid brightness reversion" was evaluated by measuring the brightness loss after the sheet had been conditioned at 23°C and 50% relative humidity, sealed in a polyethylene bag, kept at 70°C for 64h and finally removed from the bag and allowed to temperate at room temperature for at least 1 h. The brightness reversion was reported as the difference in ISO brightness units before and after reversion treatment.

### Example 1

The results after bleaching the pulp according to the invention and the reference are set out in table 2. pH and chlorine dioxide distribution in the stages D0, D1, and D2 were varied as set out in table 2.

**Table 2: Results of different modifications of the standard ECF sequence**

| Bleaching Approach | D1-D2 H | D1-D2 Temp. °C | D0/D1/D2 Distribution % of total chargeness | Bright ness % ISO | Humid Brightness Reversion ISO units |
|---|---|---|---|---|---|
| Reference | 3.0-6.1 | 90-90 | 56/41/3 | 90.5 | 14.4 |
| Invention | 3.0-3.0 | 90-90 | 45/45/10 | 90.0 | 10.5 |

In table 2, the effect of the final pH in the D2 stage and the distribution of chlorine dioxide charge in stages D0, D1, and D2 is shown, as well as humid brightness reversion. The humid reversion was reduced from 14.4 in the reference to 10.5 units according to the invention, thus a considerable improvement.

## Claims

1. Process of bleaching pulp derived from an alkaline pulping process having a hexenuronic acid content prior to the final bleaching stage from 1 to 80 mmol/kg dry pulp, said process comprising three chlorine dioxide stages D0, D1, and D2, wherein the chlorine dioxide charges based on the total chlorine dioxide charge in
a) D0 is from 40 to 60 %;
b) D1 is from 30 to 55 %;
c) D2 is from 4 to 20 %, and wherein the final chlorine dioxide stage D2 is performed at a pH from 2 to 3.5.

2. Process according to claim 1, wherein the hexenuronic acid content is from 5 to 25 mmol/kg dry pulp.

3. Process according to claim 1 or 2, wherein the hexenuronic acid content is from 5 to 15 mmol/kg dry pulp.

4. Process according to any of claims 1-3, wherein the final chlorine dioxide stage is performed at a pH from 2 to 3.4.

5. Process according to any one of claims 1-4, wherein the temperature of the final chlorine dioxide bleaching stage ranges from 85 to 100 °C.

6. Process according to any of claims 1-5, wherein the final chlorine dioxide stage is performed at a pH from 2 to 3.3.

7. Process according to any one of claims 1-6, wherein the chlorine dioxide charge in a) D0 is from 45 to 55 %, b) D1 is from 35 to 50 %, and c) D2 is from 5 to 15 %.

8. Process according to any one of claims 1-7, wherein the chlorine dioxide charge in a) D0 is from 45 to 50 %, b) D1 is from 40 to 50 %, and c) D2 is from 5 to 12 %.

9. Process according to any one of claims 1-8, wherein the temperature of the final chlorine dioxide bleaching stage ranges from 85 to 100°C.

10. Bleached pulp obtainable by the process as defined in any one of claims 1 to 9.

## Patentansprüche

1. Verfahren zum Bleichen von Zellstoff, der aus einem alkalischen Kochprozess stammt und vor dem abschließenden Bleichungsschritt einen Hexenuronsäuregehalt von 1 bis 80 mmol/kg trockenen Zellstoffs aufweist, wobei das Verfahren drei Chlordioxidschritte D0, D1, und D2 umfasst, wobei die Chlordioxidbeschickung basierend auf der Gesamtchlordioxidbeschickung bei
a) D0 von 40 bis 60 % beträgt;
b) D1 von 30 bis 55 % beträgt;
c) D2 von 4 bis 20 % beträgt, und wobei der abschließende Chlordioxidschritt D2 bei einem pH-Wert von 2 bis 3,5 durchgeführt wird.

2. Verfahren gemäß Anspruch 1, wobei der Hexenuronsäuregehalt von 5 bis 25 mmol/kg trockenen Zellstoffs beträgt.

3. Verfahren gemäß Anspruch 1 oder 2, wobei der Hexenuronsäuregehalt von 5 bis 15 mmol/kg trockenen Zellstoffs beträgt.

4. Verfahren gemäß einem der Ansprüche 1 - 3, wobei der abschließende Chlordioxidschritt bei einem pH-Wert von 2 bis 3,4 durchgeführt wird.

5. Verfahren gemäß einem der Ansprüche 1 - 4, wobei die Temperatur des abschließenden Chlordioxidbleichungsschritts im Bereich von 85 bis 100°C liegt.

6. Verfahren gemäß einem der Ansprüche 1 - 5, wobei der abschließende Chlordioxidschritt bei einem pH-Wert von 2 bis 3,3 durchgeführt wird.

7. Verfahren gemäß einem der Ansprüche 1 - 6, wobei die Chlordioxidbeschickung bei a) D0 von 45 bis 55 % beträgt, b) D1 von 35 bis 50 % beträgt, und c) D2 von 5 bis 15 % beträgt.

8. Verfahren gemäß einem der Ansprüche 1 - 7, wobei die Chlordioxidbeschickung bei a) D0 von 45 bis 50 % beträgt, b) D1 von 40 bis 50 % beträgt, und c) D2 von 5 bis 12 % beträgt.

9. Verfahren gemäß einem der Ansprüche 1 - 8, wobei die Temperatur des abschließenden Chlordioxidbleichungsschritts im Bereich von 85 bis 100°C liegt.

10. Gebleichter Zellstoff, erhältlich durch das in einem der Ansprüche 1 bis 9 definierte Verfahren.

## Revendications

1. Procédé de blanchiment de pâte dérivé d'un procédé de mise en pâte alcalin ayant une teneur en acide hexénuronique avant l'étape finale de blanchiment de 1 à 80 mmol/kg de pâte sèche, ledit procédé comprenant trois étapes au dioxyde de chlore, D0, D1 et D2, dans lequel la charge en dioxyde de chlore basée sur la charge totale en dioxyde de chlore dans
a) D0 est de 40 à 60 % ;
b) D1 est de 30 à 55 % ;
c) D2 est de 4 à 20 %, et dans lequel l'étape finale au dioxyde chlore D2 est effectuée à un pH de 2 à 3,5.

2. Procédé selon la revendication 1, dans lequel la teneur en acide hexénuronique est de 5 à 25 mmol/kg de pâte sèche.

3. Procédé selon la revendication 1 ou 2, dans lequel la teneur en acide hexénuronique est de 5 à 15 mmol/kg de pâte sèche.

4. Procédé selon l'une quelconque des revendications 1 à 3, dans lequel l'étape finale au dioxyde de chlore est effectuée à un pH de 2 à 3,4.

5. Procédé selon l'une quelconque des revendications 1 à 4, dans lequel la température de l'étape finale de blanchiment au dioxyde de chlore va de 85 à 100 °C.

6. Procédé selon l'une quelconque des revendications 1 à 5, dans lequel l'étape finale au dioxyde de chlore est effectuée à un pH de 2 à 3,3.

7. Procédé selon l'une quelconque des revendications 1 à 6, dans lequel la charge en dioxyde de chlore dans a) D0 est de 45 à 55 %, b) D1 est de 35 à 50%etc)D2estde5à15%.

8. Procédé selon l'une quelconque des revendications 1 à 7, dans lequel la charge en dioxyde de chlore dans a) D0 est de 45 à 50 %, b) D1 est de 40 à 50%etc)D2estde5à12%.

9. Procédé selon l'une quelconque des revendications 1 à 8, dans lequel la température de l'étape finale de blanchiment au dioxyde de chlore va de 85 à 100 °C.

10. Pâte blanchie pouvant être obtenue par le procédé tel que défini dans l'une quelconque des revendications 1 à 9.
